

May 13, 1947.

W. F. FILBERT

2,420,306

BLASTING CAP PRIMER COMPOSITION

Filed Jan. 10, 1942



*William F. Filbert*

INVENTOR

BY *Thos. A. Wilson*  
ATTY.

## UNITED STATES PATENT OFFICE

2,420,306

## BLASTING CAP PRIMER COMPOSITION

William F. Filbert, Woodbury, N. J., assignor to  
 E. I. du Pont de Nemours & Company, Wil-  
 mington, Del., a corporation of Delaware

Application January 10, 1942, Serial No. 426,319

6 Claims. (Cl. 52—4)

**1**

This invention relates to a new and improved blasting cap, and more particularly to caps containing a novel explosive charge of desirable properties.

It is well-known that the blasting caps of the prior art, and the explosive charges for the same have certain definite limitations and disadvantages. In particular, those skilled in the art are ready to recommend any improvements from the standpoint of safety properties.

An object of the present invention is a new and improved blasting cap containing a novel explosive charge. A further object is a blasting cap containing a new type of charge and characterized by improved safety properties. Additional objects will be disclosed as the invention is described further hereinafter.

I have found that the foregoing objects are accomplished when I employ as an explosive charge in a blasting cap a nitrated amide of a hydroxy aliphatic acid. Preferably, this compound will be used as a primary charge, but it may also function as base charge or as a portion of the ignition composition.

A number of amides of hydroxy aliphatic acids yield nitration products of attractive properties. As examples of such nitrated amides of hydroxy monocarboxylic acids I may cite the preparation of N-nitro-N-methyl hydroxyacetamide nitrate from N-methyl hydroxyacetamide



from  $[\text{CH}_2(\text{OH})\text{—CO—NH—CH}_3]$ ; N-ethanol hydroxyacetamide dinitrate from N-ethanol hydroxyacetamide



from  $[\text{CH}_2(\text{OH})\text{—CO—NH—CH}_2\text{—CH}_2\text{OH}]$ ; N-methyl gluconamide pentanitrate from N-methyl gluconamide



from  $[\text{CH}_2(\text{OH})\text{—(CHOH)}_4\text{—CO—NH—CH}_3]$ ; N-ethanol gluconamide hexanitrate from N-ethanol gluconamide



from

**2**

gluconamide pentanitrate from gluconamide



from



Likewise from aliphatic dicarboxylic acids may be prepared N,N'-dinitro-N,N'-dimethyl oxamide from dimethyl oxamide  $[\text{—CO—N}(\text{NO}_2)\text{—CH}_3]_2$  from  $[\text{—CO—NH—CH}_3]_2$ ; N,N'-diethanol oxamide dinitrate from N,N'-diethanol oxamide



from



N,N'-dinitro-N,N-dimethyl tartramide dinitrate from N,N'-dimethyl tartramide



from



N,N'-dimethyl mucamide tetranitrate from N,N'-dimethyl mucamide



from



N,N'-diethanol mucamide hexanitrate from N,N'-diethanol mucamide



from



and others. In the case of the derivatives of the dicarboxylic acids, however, I find it desirable to limit my invention to the nitration products of amides of aliphatic hydroxy dicarboxylic acids containing more than two hydroxyl groups.

It is well recognized in the literature that carbonic acid is not a true hydroxy acid. Accordingly reference to acids in the present application does not include carbonic acid.

My invention may be understood further by reference to the accompanying drawing, which is to be taken by way of illustration only and not as limiting the scope of said invention. In the

drawing, 1 represents a blasting cap shell of suitable metal and of the customary cylindrical shape, 2 designates a base charge of pentaerythritol tetranitrate, 3 a primary charge of N-methyl gluconamide pentanitrate, and 4 an ignition charge comprising a grained mixture of diazodinitrophenol with N-methyl gluconamide pentanitrate. This ignition mixture may be fired by the spit of a fuse inserted into the upper part of the cap shell and crimped tightly thereto, or alternatively by means of a hot wire as in the conventional electric blasting caps, in which case the mouth of the shell is closed about leg wires by any conventional closure means.

The following examples show specific embodiments of the application of my invention to blasting caps, the compositions shown giving satisfactory execution. Conventional ignition charges were employed in all cases where the type is not indicated.

invention. While in many cases it will be employed in connection with caps adapted for ignition by means of a fuse, it is applicable also for electric blasting caps, delay caps, and the like. 5 I intend to be limited therefore only by the following patent claims.

I claim:

1. A blasting cap containing a base charge of pentaerythritol tetranitrate, a primer charge 10 comprising N-methyl gluconamide pentanitrate, and an ignition composition comprising diazo- dinitrophenol grained with N-methyl gluconamide pentanitrate.

2. A blasting cap containing a base charge of 15 any secondary explosive, a primer charge comprising a nitrated amide of an acid from the group consisting of the aliphatic hydroxy monocarboxylic acids and those aliphatic hydroxy dicarboxylic acids containing more than two hydroxyl 20 groups and an ignition composition comprising

|   | Base Charge                                | Wt.,<br>Grains | Primary Charge                     | Wt.,<br>Grains | Ignition Charge                                                               |
|---|--------------------------------------------|----------------|------------------------------------|----------------|-------------------------------------------------------------------------------|
| 1 | N-nitro-N-methyl hydroxyacetamide nitrate. | 4              | Lead azide-----                    | 1.0            |                                                                               |
| 2 | N-methyl gluconamide pentanitrate.         | 4              | Diazodinitrophenol-----            | 2.5            |                                                                               |
| 3 | Gluconamide pentanitrate-----              | 4              | Lead azide-----                    | 2.0            |                                                                               |
| 4 | N,N'-dimethylmucamide tetranitrate.        | 4              | do-----                            | 1.0            |                                                                               |
| 5 | Pentaerythritol tetranitrate.              | 4              | N-methyl gluconamide pentanitrate. | 1.0            | Diazodinitrophenol grained with nitromannite—1 grain.                         |
| 6 | do-----                                    | 4              | Same-----                          | 1.5            | Diazodinitrophenol grained with N-methyl gluconamide pentanitrate—1.5 grains. |

I find that the nitrated amides of hydroxy aliphatic acids as disclosed in the foregoing give desirable results when used as cap charges. They may be employed as base charges with good effect and I find the compound N-methyl gluconamide pentanitrate to be a particularly satisfactory material. When employed as a primary charge in a fuse cap above a base charge of pentaerythritol tetranitrate. I find said cap to have outstanding properties, particularly when a grained blend of said N-methyl gluconamide pentanitrate and diazodinitrophenol is employed as ignition agent.

In my copending application Serial No. 424,903, filed Dec. 30, 1941, I have claimed these amides as new chemical and explosive compounds.

I have described my invention at length in the foregoing, but it will be understood that many variations may be introduced in compositions and details without departure from the scope of said

diazodinitrophenol grained with one of said nitrated amides.

3. A blasting cap containing a base charge of 35 a secondary explosive, a primer charge comprising a nitrated amide of an acid from the group consisting of aliphatic hydroxy monocarboxylic acids and those aliphatic hydroxy dicarboxylic acids containing more than two hydroxyl groups, 40 and an ignition composition disposed above said primer charge.

4. The blasting cap of claim 3 wherein said primer charge comprises N-methyl gluconamide pentanitrate.

5. The blasting cap of claim 3 wherein said primer charge comprises N-nitro-N-methyl hydroxyacetamide nitrate.

6. The blasting cap of claim 3 wherein said primer charge comprises N,N'-dimethyl mucamide tetranitrate.

WILLIAM F. FILBERT.